

## UNITED STATES PATENT OFFICE.

LE BARON W. KINNEY, OF CLEVELAND, AND GEORGE H. BIERMAN, OF EAST CLEVELAND, OHIO, ASSIGNEES TO THE WHITE MOTOR COMPANY, OF CLEVELAND, OHIO, A CORPORATION OF OHIO.

## PROCESS OF HEAT TREATING STEEL.

No Drawing.

Application filed September 27, 1928. Serial No. 188,117.

This invention relates to the process of treating steel which is to be subjected to heat treatment in an electric furnace and particularly to an improved method of heat treating steel gears and similar articles having hardened machined surfaces.

It has been found that steel articles such as gears which have been heat treated in an electric furnace are relatively softer on their outer surfaces than articles heat treated in gas fired or oil burning furnaces. This softened surface condition does not occur in gas and oil fired furnaces as the carbonaceous gases to which the gears are subjected during heat treatment preserve the carbon content of the steel. In the electric furnace, however, the steel is exposed to atmospheric air the oxygen in which decarburizes the outer surface of the gear to a depth exceeding the commercial and practical grinding allowance usually employed in machine shop practice. The result of this deleterious surface decarbonization is that the shape of the tooth or wearing face of the article which has been so carefully designed and formed will be rapidly worn away when the article is put into service unless, in the manufacture, a sufficient amount of grinding or machining stock is allowed to assure the removal of the softened surface. The latter practice obviously increases the production time and cost and furthermore, is uncertain of result as there is no uniformity in the depth of the decarbonization.

For instance in a cam of irregular formation the most practical grinding tolerance, according to the particular design, may be five thousandths of an inch and this may be an adequate allowance for the major portions of the cam, but at the peak of the cam, where the greatest wear usually occurs, the steel may be decarburized to a depth of ten to twelve thousandths while all other surfaces are only softened one or two thousandths in depth. Moreover there is still a further uncertainty as to what the depth of the decarbonization may be, this variation residing in different allotments of steel of the same grade wherein some specimens are found to vary from five to ten thousandths more than others under identical treatment.

The object of this invention is to produce steel gears and similar objects which will

have hardened outer surfaces after heat treatment in an electric furnace.

In carrying out the invention, a steel gear which may be considered as illustrative for the purpose of describing the invention, is first carbonized and machined, then coated with a material characterized by its impregnability by decarbonaceous gases at a temperature of approximately 1400° F., also by its ability to readily adhere to the steel at the instance of application and throughout the period of heat treatment. It is immaterial whether or not the material employed becomes fused or fluidic at the temperature to which the gear is subjected provided that it does not become porous or flow from any portion of the gear while in the furnace or during its removal therefrom. It is essential that the material used to coat the gear be capable of withstanding high temperatures for a period of forty to sixty minutes without disintegration of such molecular rearrangement as would expose the gear to the oxygen laden contents of the electric furnace as this period of time is sufficient to soften the gear surface. It is preferable that one of the qualities of the coating material be such that no physical or chemical changes take place which would destroy the adhesion of the coating material or affect its heat resisting properties between the time the gear is coated and the time at which it is placed in the furnace. The advantage of this quality will be seen where the progress of the process is interrupted and it is found to be more convenient to apply the coating one day and to heat treat the gear some time later. An example of such a material is sodium tetra borate or boric anhydride although other materials or the combination of various materials having the above characteristics may be used.

The preferred practice of applying the material is to submerge the gear in a solution of water and borax to which an adulterant of diatomaceous earth or finely comminuted particles of silica may be added to thicken the solution and assure a thorough and even coating. When an adulterant is employed it has been found advantageous to maintain this material in suspension by agitating the solution with a suitable stirring mechanism or by boiling it. A solu-

tion comprising the above ingredients has been found to be the most successful when proportioned with 55% water, 30% borax, and 15% diatomaceous earth or kieselguhr. 5 This solution affords not only a heavy impregnable coating but in addition has the advantage of maintaining its liquefied state from day to day without appreciable change.

Various modifications may be made in the 10 mode of applying the coating or insulating material before heat treatment such as dusting powdered borax on an article which has been pre-heated to the melting point of borax and permitting the borax thus deposited to become fused then to rotate the article until the surfaces are entirely coated. This method while successful on some forms of work is not entirely dependable as the powdered borax fuses so readily that it is apt 15 20 to flow away from the surfaces which are contiguous with the greatest mass of steel.

Another method of applying the coating is to submerge the gear into a molten mixture of borax in which powdered stone or 25 plaster of Paris is held in suspension by any suitable means.

After the gear is coated it may be placed in an electric furnace and heat treated and quenched according to the accepted practice 30 for the particular grade of steel employed

and thereafter the coating material may be removed by sand blasting or in a pickling process of the usual type.

Although the preferred form of applying the coating is the method first described, it 35 is to be understood that the invention is not limited to the precise mode of applying the coating nor to the specific materials above described, but includes all materials having the same or concomitant qualities, characteristics and properties.

Having thus described the invention, what is claimed and desired to be secured by Letters Patent, is:

1. The composition for preventing decarbonization while heat treating comprising 45 55 percent water, 15 percent kieselguhr, and 30 percent borax.

2. A composition for preventing decarbonization during heat treatment consisting 50 entirely of kieselguhr, water, and borax.

3. A composition for preventing decarbonization during heat treatment comprising substantially one part kieselguhr, two parts borax, and four parts water. 55

In testimony whereof we hereunto affix our signatures this 18th day of September, 1926.

LE BARON W. KINNEY.  
GEORGE H. BIERMAN.